

## UNITED STATES PATENT OFFICE

HANS WEIGEL, OF ECKING, GERMANY

## ROLLING PROCESS

No Drawing. Application filed February 24, 1930, Serial No. 431,048, and in Germany February 23, 1929.

My invention relates to improvements in rolling processes and more particularly in processes which are combined with a refining process. As now practised the process of refining wire, for example by chilling the same by means of water, oil or the like, is performed at the end of the rolling operation. The object of the improvements is to provide a process which results in a material of improved properties, and with this object in view my invention consists in performing the said refining operation in the course of the rolling operations, the refining operation being followed by one or more rolling operations. In the preferred form of the process I subject the material being rolled to a plurality of successive refining operations each followed by one or more rolling operations, and in some cases I perform a chilling operation after each rolling operation. I have found that the material treated by my improved process is materially refined, because the mechanical operation or operations following the chilling assist the formation of a sorbitic structure of the metal.

The rolled metal is refined in the manner described for the purpose of rendering the same suitable for further treatment in a cold state, for example by drawing, and for other purposes. Thus the metal is passed through a plurality of roll-trains after once chilling.

It will be seen from the foregoing that the process consists in rolling a steel wire to be wire-drawn. The steel wire is subjected to a plurality of rolling operations to cause a change in the sorbitic structure of the metal by quenching the steel wire immediately upon being rolled and then subjecting the quenched steel wire to another rolling operation immediately after the aforesaid quenching. By this rolling and quenching there is a refinement in the composition of the steel to produce a sorbitic structure to adapt it to a subsequently cooled wire drawing process.

In some cases I subject the metal to a plurality of refining operations after one rolling operation and prior to a second rolling operation.

I claim:

50 In the process of rolling steel wire to be

wire-drawn in which the steel wire is successively subjected to rolling operations, the method of forming a sorbitic structure in steel wire for refining it during the rolling process, which consists in quenching the steel wire while heated immediately after one rolling operation during the rolling process, and subjecting the heated quenched steel wire to another rolling operation immediately after the quenching, for refining the steel wire to produce a sorbitic structure therein, thereby adapting it to subsequent cold wire drawing.

In testimony whereof I hereunto affix my signature.

HANS WEIGEL.

65

70

75

80

85

90

95

100